

## UNITED STATES PATENT OFFICE

2,017,804

## DELUSTERED ARTIFICIAL SILK YARN

Frederick W. Koster, Meadville, Pa., assignor to  
The Viscose Company, Marcus Hook, Pa., a  
corporation of Pennsylvania

No Drawing. Application September 16, 1931,  
Serial No. 563,233

2 Claims. (Cl. 28—1)

The object of my invention is to produce an improved delustered artificial silk thread or yarn, and more particularly cellulose acetate yarn and this I accomplish by the use of chlorinated naphthalene which is commercially known as halowax. It is a creamy-white wax insoluble in water, but soluble in certain solvents. This ingredient I combine with the cellulose acetate spinning solution by the use of the same solvent as is used to produce the spinning solution of cellulose acetate.

In making up a spinning solution for the evaporative process, the cellulose acetate is dissolved as usual in acetone containing approximately 2.5% water. Before this process of solution has been completed, I add to the acetate solution and mix thoroughly with the latter halowax which has been dissolved in acetone, the same solvent as used for the spinning solution. The amount of halowax is preferably about 12% of the cellulose acetate used, and it is dissolved in about three times its own weight of acetone. These two solutions are thoroughly mixed together, giving a spinning solution in which no solid particles are visible, except as ordinarily occur in the regular operation. If desired, the required amount of halowax may be dissolved in the whole of the acetone charge before adding the cellulose acetate or else the halowax and cellulose acetate may be dissolved simultaneously in the total acetone charge.

The process of evaporative spinning causes a solidification of both the cellulose acetate and the halowax simultaneously, as the common solvent disappears. It is believed that the particles of halowax are formed inside the particles of cellulose acetate and cause the desired delustered appearance by a dispersion or refraction of light passing through the mass. The percentage of chlorinated naphthalene is preferably limited to between 5% and 20% of the weight of cellulose acetate, because less than 5% chlorinated naphthalene in the yarn does not give an appreciable delustering effect and more than 20% materially weakens the fibers without giving any apparent increase in the degree of delustering.

The resulting product is an artificial silk thread delustered by having fine particles of chlorinated naphthalene immersed in and distributed throughout the mass of the thread.

I claim as my invention:

1. As a new article of manufacture, delustered artificial silk thread having immersed in and distributed throughout its mass material fine particles of chlorinated naphthalene.
2. As a new article of manufacture, delustered cellulose acetate thread having immersed in and distributed throughout its mass material fine particles of chlorinated naphthalene.

FREDERICK W. KOSTER. 30